

Nov. 16, 1943.

H. FINK ET AL

2,334,615

CONTINUOUS SPINNING OF CELLULOSE SOLUTIONS IN STRONG MINERAL ACIDS

Filed Aug. 28, 1939

3 Sheets-Sheet 1

Fig. I



Inventors  
Heinrich Fink  
Gustav Rath  
Richard Hofstadt  
By Their Attorneys

*Stahl and Joslin*

Nov. 16, 1943.

H. FINK ET AL

2,334,615

CONTINUOUS SPINNING OF CELLULOSE SOLUTIONS IN STRONG MINERAL ACIDS

Filed Aug. 28, 1939

3 Sheets-Sheet 2

Fig. II



Inventors  
Heinrich Fink  
Gustav Rath  
Richard Hofstadt  
By Their Attorneys  
*Hofstadt and Joskin*

Nov. 16, 1943.

H. FINK ET AL

2,334,615

CONTINUOUS SPINNING OF CELLULOSE SOLUTIONS IN STRONG MINERAL ACIDS

Filed Aug. 28, 1939 3 Sheets-Sheet 3

Fig. III



Inventors:  
Heinrich Fink  
Gustav Rath  
Richard Hofstadt

By Their Attorneys

*and Joslin*

## UNITED STATES PATENT OFFICE

2,334,615

## CONTINUOUS SPINNING OF CELLULOSE SOLUTIONS IN STRONG MINERAL ACIDS

Heinrich Fink, Gustav Rath, and Richard Hofstadt, Wolfen, Kreis Bitterfeld, Germany; vested in the Alien Property Custodian

Application August 28, 1939, Serial No. 292,254  
In Germany August 30, 1938

4 Claims. (Cl. 18—54)

It is known to dissolve cellulose in mineral acids such as sulfuric acid and phosphoric acid and to work up the solutions to form artificial shaped bodies such as fibers or films.

The solutions of cellulose in strong mineral acids are distinguished from cellulose solutions in ammoniacal copper oxide and quaternary bases as well as from viscose by a much higher viscosity with the same content of cellulose, and by the rapid degradation to which the cellulose is subject in strong mineral acid solutions.

These properties combinedly render the production and working up of useful spinning solutions very difficult. Owing to the high viscosity, the mixing of the mass to homogeneity is very slow, being slower, the larger the batch. Deaeration of the highly viscous mass is impossible. If the solution is produced in a vacuum kneader it is impossible to transfer the solution to the spinning reservoir without introducing fresh air into the solution. On the other hand owing to the rapid degradation of the cellulose a reduction of the time taken in dissolving the cellulose and in working up the solution is desirable.

It is, indeed possible to reduce the rate of degradation of the dissolved cellulose by keeping the solution at a low temperature, but apart from the expense involved this possibility is limited in practice by the fact that the solution becomes more viscous the lower the temperature.

It has further been proposed to reduce the rate of degradation of the dissolved cellulose by reducing the concentration of the solvent acid below the concentration necessary for dissolution of the cellulose fibers by addition of a more dilute acid or of another diluent after the cellulose has been dissolved. Apart from the fact that the content of cellulose of the solution is thereby diminished to an undesirable extent, the gradation of the cellulose in this so-called "meta-stabilized" solution is much more rapid than appears from the viscosity curve of the solution.

In working up successive batches in the usual manner the difficulty arises that the solution exhibits from the outset an undesirable rate of degradation of the cellulose and that the degree of degradation varies greatly from the beginning to the end of a batch, a sudden change in the degree of degradation occurring at the beginning of each batch. Owing to the great viscosity of the solution one batch cannot be completely removed from the spinning reservoir before the next batch is introduced, so that residues of previous batches in an advanced state of degradation are mixed with the fresh batch. Thus the solution reaching

the spinning nozzle continuously alters its properties, thereby rendering the production of uniform products of high value impossible. Moreover it is practically impossible to make the solutions to be worked up free from air.

The present invention overcomes these difficulties by making use of the known property of cellulose of swelling strongly in mineral acids of a certain concentration, whereby the union between the fibers is so loosened that there is produced a suspension of fibers of a pasty consistency which can easily be made to flow like a liquid by means of pumps, worms, pistons and the like. We have found that in this suspension of fibers the degradation of the undissolved cellulose is so slow that it is of no practical significance.

Reference is made to the accompanying drawings in which:

Figure 1 shows diagrammatically a sectional view of an apparatus for carrying the invention into effect.

Figure 2 is a diagrammatic longitudinal section of an apparatus comprising pressure worms as a means for feeding the suspension and solution of cellulose, and

Figure 3 is a diagrammatic longitudinal section of a modification of the apparatus shown in Figure 2.

By the invention a suspension of cellulose in a strong mineral acid of which the concentration is nearly but not quite sufficient to dissolve the cellulose is fed continuously to the spinning nozzle and there is added to the suspension on its way to the spinning nozzle sufficient strong mineral acid to dissolve the cellulose when uniformly mixed with the suspension. By moving the suspension slowly forward at a uniform rate by pressure and thoroughly mixing with the acid by means of a stirring device, the cellulose dissolves rapidly. Preferably a dissolving chamber is arranged in the path to the spinning nozzle, and there may advantageously be a further chamber of a similar kind for homogenizing the solution, whereupon the solution can, if necessary, be passed through a filter which is connected directly with the nozzle for producing fibers, foils, tubes or the like.

The only discontinuous process consists in the production of relatively small batches of the suspension, since in this phase there is no danger of degradation at the proper temperature, for instance 0° C. On the other hand once the suspension has entered the apparatus as much cellulose is dissolved per unit time as leaves the apparatus in the same time. Since the dissolution is

rapid the quantity of solution present in the apparatus can be kept very small. For example the total capacity of an apparatus for dissolving 100 kg. of cellulose in 24 hours need not amount to more than 3 liters, even if chambers of capacity 2-3 liters for dissolving the cellulose and homogenizing the solution are provided. This ensures that the time from the entry of a cellulose molecule into solution until its exit from the apparatus is only a few minutes. This time is so short that with moderate cooling, for example to 0° C., there is less degradation of the cellulose in the mineral acid than occurs for instance in the technical working of the viscose or cuprammonium process. In consequence meta-stabilization of the solution, which of course in cases in which it is required could be introduced into the process without difficulty, can be entirely dispensed with.

If the invention is carried out in such a manner that the suspension of cellulose in a mineral acid is de-aerated instead of the cellulose solution ready for spinning, a completely air-free cellulose solution is obtained in which formation of air bubbles is impossible owing to the filling of the space by the mass.

The deaeration of the suspension is naturally produced more rapidly and completely the poorer it is in cellulose, the degree of swelling of the cellulose being assumed to be in each case the same. For many purposes, however, it is solutions with the highest possible content of cellulose and the lowest possible content of swelling acid that are required. Since the batches containing the minimum of swelling acid are too stiff to be well evacuated the process is so carried out that the suspension is formed with an excess of swelling acid and is deaerated, whereupon the excess is pressed off in the apparatus itself, before entry of the mass into the dissolving chamber. This may be done for example by forming the feeding device before the dissolving chamber as a pressure worm. The degree of pressure depends on the degree of swelling of the cellulose which is determined by the concentration of the swelling acid and, for instance, when using sulfuric acid, increases especially rapidly in the region of 58-60 per cent sulfuric acid.

Referring now to Figure 1, 1 denotes two similar pressure-tight cylinders of acid-resisting material having removable lids 2. Machined pistons 3 having rods 4 of which the lower parts are screw-threaded, are adapted to be moved by the driving wheels 5, in the cylinders 1. The means for driving the wheels 5 are the motors M and gears 5a. The cylinders are provided at their upper ends with pipes having cocks 6 and connected with vacuum apparatus. In order to prevent air from being sucked in through lack of tightness of the stuffing boxes and the pistons a branch pipe 18 may be connected with the lower ends of the cylinder.

During upward movement of either piston the contents of the cylinder 1 is pressed through a pipe provided with a cock 7 into the cylindrical dissolving chamber 8 in which an eccentrically arranged roller 9 rotates. At the same time the calculated quantity of mineral acid of the concentration required for dissolving the cellulose is pumped into the chamber 8 from a reservoir by means of a pump 10. Preferably the entries of the dissolving acid is distributed over the whole circumference of the chamber 8 by means of a circular pipe with a large number of perforations. By the rotating eccentric roller 9 there is added to the forward motion of the mass produced by

the piston 3 a circular motion which brings about a thorough admixture of the suspension with the dissolving acid, so that a clear cellulose solution leaves the chamber 8 through the pipe 11. The solution after passing, if necessary, through a filter 17 is fed by metering pumps 12 to the spinning nozzles.

In this apparatus the solution is fed uniformly forward by the propulsion of the pistons 3. The suspension is supplied by removing the lid 2 of the cylinder 1 whose piston 3 is for the time being in its lowest position and filling the cylinder with suspension. When the lid is screwed on the cylinder is evacuated while the other piston 3 makes its working stroke. When the latter reaches its highest position it is stopped and at the same time the other piston 3 comes into operation, the cocks 7 being reversed. In this manner the suspension continually enters the chamber 8 and passes to the spinning nozzles through the pipe 11 while the cylinders 1 are charged discontinuously.

In the apparatus shown in Figure 2 the cellulose suspension is likewise fed alternately to at least two cylinders 1 and is deaerated through pipes provided with cocks 6 before proceeding further. In this case the cylinders have no lids but are filled by entirely removing the plungers 3. The role of the cylinders 1 and plungers 3 is, however, in this case only to supply the feeding worm 13 by way of the valve 1a with the suspension under a steady weak pressure. The cylinders 1 and pistons 3 can in this case be much weaker than those of Figure 1 since the actual feeding of the suspension is performed by the driven worm 13. The latter feeds the suspension into the dissolving chamber 14, which is likewise provided with a feeding worm and is supplied with dissolving acid from the pipe 10. To enhance the mixing effect a counter-worm as shown in Figure 3 (reference numerals 22-24) may also be provided in the dissolving chamber. After leaving the dissolving chamber the solution passes to two or more homogenizing worms 15 which feed the solution through pipes 11 to the spinnerets.

Figure 3 shows apparatus which is suited for the production of air-free solutions especially rich in cellulose. Only one charging container 1 with stirrer 1a and deaerating connection 6 is shown the other or others being assumed to lie outside the plane of the paper behind container 1 a reversal valve such as 1a in Figure 2 being provided between them. Into the container 1 the suspension is fed with an excess of swelling acid while stirring and is then deaerated. The mass is in this case so thin that it runs under its own head into the chamber provided with the worm 13, the containers 1 being again used alternately. The worm 13 in this case acts as a pressure worm as is indicated by its tapering form. The walls of the press-chamber are hollow, the wall 16 being perforated to allow the excess of swelling acid to be extruded into the tank 25 where it can be collected and returned to the mixer in which the cellulose is swollen. The suspension having a reduced content of swelling acid is then fed into the dissolving chamber 22, to which acid is supplied from the pipe 10. The dissolving chamber 22 is provided with a kneading pump of the usual construction having two geared worms 23 and 24. The mass is then fed through the homogenizing worms 15 and pipes 11 to the spinnerets.

The apparatus of Figure 1 is used especially in

those cases in which no particularly high output is required. The apparatus of Figures 2 and 3 on the other hand work more quickly owing to the distribution of pressure over the whole apparatus, and are especially advantageous in those cases in which a large output is required.

In all cases it is advantageous to provide the whole apparatus from the charging containers to the spinnerets with a cooling jacket through which brine at about 0° C. is circulated. The jacket is not shown in the drawings for the sake of clarity.

The invention is illustrated by the following examples:

*Example 1*

With every 3 kg. of cellulose (air-dry) there are stirred, while cooling to 0° C., 30 kg. of sulfuric acid containing 59.0 per cent of H<sub>2</sub>SO<sub>4</sub> and the mixture is fed into the similarly cooled cylinder 1 shown in Figure 1 or Figure 2 and evacuated. From there the suspension is fed continuously during about 30 minutes by means of the piston 3 into the dissolving chamber 8, which is continuously supplied by means of the metering pump 10 with 11 kg. of sulfuric acid containing 75 per cent of H<sub>2</sub>SO<sub>4</sub> for every cylinder-full of suspension. While the full cylinder 1 is being emptied the other cylinder is filled and evacuated and the process is then repeated after reversal of the valves. The solution takes place at about 0° C. From the outlet of the chamber 8 there emerges continually a completely clear solution which can be spun in the usual manner to fibers or otherwise worked up.

*Example 2*

4.5 kg. of cellulose (air-dry) in 45 kg. of sulfuric acid containing 59.5 per cent of H<sub>2</sub>SO<sub>4</sub> are introduced into the container shown in Figure 3 and stirred at 0° C. The mixture is then evacuated. The containers are used alternately. After evacuation the batch is run into the chamber containing the pressure worm 13 which expresses 16 kg. of swelling acid per batch, so that the mass enters the dissolving chamber with a content of 29 kg. of swelling acid to 4.5 kg. of cellulose. 9.5 kg. of sulfuric acid containing 75 per cent of H<sub>2</sub>SO<sub>4</sub> and cooled to 0° C. are supplied to the dissolving chamber. The solution produced contains 9.8 per cent of cellulose and 57 per cent of H<sub>2</sub>SO<sub>4</sub>.

We claim:

1. A process of continuously producing solutions of cellulose in a strong mineral acid which comprises suspending the cellulose in a mineral acid of a concentration which will cause swelling of the cellulose, but will not dissolve it, feeding said suspension continuously to an extruding device and adding to said suspension on its way to the extruding device a strong mineral acid in an amount which is necessary to dissolve the cellulose in said suspension, the amount of solution formed per time unit being kept the same as the amount of solution leaving the extruding device.
- 15 2. A process as claimed in claim 1 where the mineral acid in the suspension is sulfuric acid with a content of about 59 per cent of H<sub>2</sub>SO<sub>4</sub> and the strong mineral acid dissolving the suspension is sulfuric acid of about 75 per cent of H<sub>2</sub>SO<sub>4</sub>.
- 20 3. A process of continuously producing solutions of cellulose in a strong mineral acid which comprises suspending the cellulose in a mineral acid of a concentration which will cause swelling of the cellulose but will not dissolve it, continuously removing a part of the suspension liquid from the suspension, feeding said suspension continuously to an extruding device and adding to said suspension on its way to the extruding device a strong mineral acid in an amount which is necessary to dissolve the cellulose in said suspension, the amount of solution formed per time unit being kept the same as the amount of solution leaving the extruding device.
- 25 35 4. A process of continuously producing solutions of cellulose in a strong mineral acid which comprises suspending the cellulose in a mineral acid of a concentration which will cause swelling of the cellulose but will not dissolve it, de-aerating the suspension, feeding said suspension continuously to an extruding device and adding to said suspension on its way to the extruding device a strong mineral acid in an amount which is necessary to dissolve the cellulose in said suspension, the amount of solution formed per time unit being kept the same as the amount of solution leaving the extruding device.

HEINRICH FINK.  
GUSTAV RATH.  
RICHARD HOFSTADT.